# EUROPEAN PATENT SPECIFICATION

(11) **EP 0 581 257 B1**
(45) Date of publication and mention of the grant of the patent: **18.11.1998**
(21) Application number: 93112029.9
(22) Date of filing: 28.07.1993
(51) Int. Cl.: G03G 9/00, G03G 9/08

(54) **Electrophotographic magnetic toner for development an image and a method of producing the same**
Elektrophotographischer magnetischer Toner zur Entwicklung eines Bildes und Verfahren zur dessen Herstellung
Toner magnétique électrophotographique pour le développement d'images et procédé pour sa fabrication

(30) Priority: 29.07.1992 JP 202191/92; 04.08.1992 JP 207773/92; 04.08.1992 JP 207774/92; 19.11.1992 JP 309956/92; 19.11.1992 JP 309957/92
(43) Date of publication of application: 02.02.1994
(73) Proprietor: MATSUSHITA ELECTRIC INDUSTRIAL CO., LTD., Kadoma-shi, Osaka-fu, 571 (JP)
(72) Inventor: Yuasa, Yasuhito, Hirakata-shi, Osaka (JP); Toyoda, Akinori, Katano-shi, Osaka (JP); Hirota, Noriaki, Higashiyodogawa-ku, Osaka-shi, Osaka (JP)
(74) Representative: Eisenführ, Speiser & Partner

(56) References cited:
- EP-A- 0 374 851
- EP-A- 0 488 789
- DE-A- 2 825 002
- DE-A- 3 809 662
- US-A- 4 221 554

## Description

### BACKGROUND OF THE INVENTION

### Field of the Invention

The present invention relates to an electrophotographic magnetic toner for use in an image development apparatus such as a copier, printer, facsimile, and the like.

### Description of the Prior Art

As a development method in an electrophotographic technique, there have been available conventionally a cascade development method, touchdown development method, jumping development method, and others. Among these methods, the cascade development as disclosed in the U.S. Patent 3,105,770 has been known as a development method in which developer is sprinkled directly onto a photoconductor. The cascade development method was used for the first time in a practical copier for electrophotography.

Further, in the U.S. Patent 3,866,574 disclosed is a development method in which mono-component toner is jumped onto a photoconductor by applying an AC bias voltage to a developing roller thereby to effect development. In this U.S. Patent, the AC bias voltage to be applied to the developing roller is used for the purpose of activating the movement of the toner, where it is described that the toner jumps to image areas and returns on the way to non-image areas on the photoconductor.

As an improvement of the AC bias application technique, there is disclosed a jumping development method in the Japanese Patent Publication 63-42256 (published in 1988). In this jumping development method, the toner is supported by a toner support member, and on the toner support member there is provided a doctor blade for regulation of a rigid body or elastic body at a minute spacing to the support member. The toner is regulated into a thin layer by the doctor blade and transferred to a developing section, where the toner is deposited on the image areas of the photoconductor with the AC bias application. The technical concept of the Japanese Patent Publication 63-42256 differs from that of the U.S. Patent 3,866,574 in that the toner is moved reciprocatingly at image areas and non-image areas.

As is known, in these development methods, the toners for use in electrostatic charge development are generally composed of resin components, coloring agents of pigments or dyes, and additive components such as plasticizers and charge control agents. As the resin components, natural resins or synthetic resins are used solely or by mixture as the case may be.

However, there has been desired a further improvement in quality of copied images and their long-term stability of image quality in recent years.

Moreover, nowadays, from a viewpoint of the earth environmental protection, it is necessary to regulate unlimited disposal of industrial wastes. It is also an important problem to recycle the wastes.

With the conventional constitutions and methods as described above, it has been well known to those skilled in the art that the cascade development is no good at reproduction of solid blacks. Another problem is involved in the cascade development that the system for the development method would be large in scale and complex in structure. Further, the developing device as disclosed in the U.S. Patent 3,866,574 has had such a drawback that high precision is required for the system, which leads to a complex structure and high cost. In the jumping development method, it has been indispensable to form an extremely uniform thin layer of a toner on a toner support member carrying a toner layer. In this method, another problem has been frequently involved that there occurs a so-called sleeve ghost development in which there remains hysteresis of the preceding image of the toner thin layer formed on the toner support member, which causes an afterimage to appear in the resulting image. The method has also a problem that a complex equipment and high cost are required disadvantageously.

Therefore, the applicant of the present invention has previously proposed a new electrophotographic system in which smaller-in-size, higher-in-performance for development can be realized without using a doctor blade. The development process in the new electro-photographic system is implemented by providing a photoconductor containing a stationary magnet, and an electrode roller having a magnet opposed to the photoconductor at a specified spacing. Thus, by this development method, it becomes possible to reproduce solid blacks with fidelity, free from occurrence of sleeve ghost, allowing the system to be further reduced in size, simplified in construction, and lowered in cost.

To improve the quality of images by using this development method, however, there is a need for even higher performance of toner properties. In this development method, since no doctor blade is provided for regulating the toner into a thin layer, the toner is transferred to the development field which is defined by a space of a narrow gap between the photoconductor and the electrode roller, without being regulated into a layer. As a result, the place and space needed to obtain a desired charge amount for the toner to be triboelectrified is restricted to only a small one, so that the toner is required to have higher charging characteristic than in conventional one. It is the fluidity and electrical resistance of a surface of toner particles which affects the toner's high charging characteristic. Fluidity can be defined by apparent density, and the surface resistance can be defined by a dielectric loss.

The fluidity of the toners used in the conventional mono-component development or two-component development has drawbacks such that non-uniformities would occur in solid-black image areas and half-tone image areas and besides background fogs would increase in non-image areas. This phenomenon can be found remarkably in toners having low fluidity. This can be attributed to the fact that toners with low fluidity cannot afford satisfactory amounts of triboelectrification due to low possibility of contact with the developing member. Moreover, there arises non-uniformities in the triboelectrification performance among individual toners, so that uniform toner chargeability cannot be obtained. On the other hand, toners keeping high fluidity exhibit uniform contactability with the developing member, so that a high level of charge amount can be obtained, in which case high-quality images can be obtained.

For enhancement of fluidity of toners, there has been taken a measure of increasing an adding amount of additives such as silicon oxide, which is a fluidity imparting agent. However, if additives of such as silicon oxide are increased in quantity, the fluidity increases with increasing amount of additives, while suspended particles of silicon oxide also increase in amount such that the silicon oxide is implanted as cores into the photoconductor by urging force of a cleaning blade, resulting in causing flaws. As a result, there would occur a phenomenon of filming that silicon oxide or toner adheres onto the photoconductor. Meanwhile, the suspended particles of silicon oxide adhere to solid black areas, bringing about white dots. In consequence, increasing the amount of silicon oxide results in disadvantages in many respects, making no solution of the problems.

Conventional magnetic toners have magnetic materials internally added in the binder resin. The toner is pulverized to be finely divided. In this process, since the magnetic material that is lower in electric resistance than the binder resin is exposed on the toner surface, therefore the charges obtained through triboelectrification are likely to leak, such that the magnetic toner encounters difficulty in obtaining large amount of charges, to a disadvantage.

As a further aspect, earth environmental protection has come up to an issue of great significance in recent years. In conventional copiers, laser printers, laser facsimiles, and the like, a toner is developed on the photoconductor in the development process and then transferred onto paper in the transfer process. In these processes, a part of the toner remains on the photoconductor. The part of the remaining toner is swept down in the cleaning process. The cleaned-off toner results in residual toner. In the conventional methods, especially in the mono-component development, the residual toner is wasted, which can not be recycled.

In recycling the residual toner swept off the photoconductor in the cleaning process for once more development, the toners in the conventional method will result in non-uniform charge distribution if the residual toner is mixed with unused toner within the developing unit, such that wrong sign toner of reversed triboelectric charge polarity increases, causing deterioration of the quality of copied images.

Further, the conventional mono-component development is implemented in the arrangement that a toner-layer doctor blade of an elastic body or the like is provided, spaced from the toner support member at a narrow gap or in slightly contact therewith, where a toner thin layer is formed on the toner support member. In this arrangement, it is likely that agglomerations of the residual toner bring about clogging in proximity to the toner-layer regulator blade, causing white voids. The residual toner may have silicon oxide buried into the toner by the pressure involved in the cleaning blade process, resulting in changes in the adhesion state of the silicon oxide or in defects or cracks of the toner. This accounts for deterioration of the fluidity of the residual toner. Such toner that has lowered in fluidity tends to bring about agglomeration. Those factors form the difficulty in realizing the recycle of toner.

The above-described situation results in not only the impossibility of effective utilization of resources, but may cause pollution of the earth environment as well. Consequently, it is a problem of great urgency to recycle the residual toner for re-utilization of resources, in terms of the earth environmental protection.

EP-A-488 789, DE-A-3809662 and DE-A-2825002 disclose electrophotographic magnetic toners. US-A-4 221 554 defines an apparatus and a method to form spherical particles of thermoplastic material.

### SUMMARY OF THE INVENTION

Accordingly, an essential objective of the present invention is to provide an improvement of a magnetic toner for use in a development method which allows the system to be further reduced in size, simplified in construction, and lowered in cost and moreover allows recycling of the residual toner, the magnetic toner having high fluidity and high chargeability in order to realize high quality of images with high image density and low background fogging, preventing filming onto a photoconductor.

Another objective of the invention is to provide a method of manufacturing the magnetic toner which is free from any lowering of toner charge amount and fluidity and free from occurrence of agglomerations even if the residual toner is recycled to be mixed with an unused one.

A further objective of the invention is to provide a magnetic toner which can be designed for prolonged life, which allows recycling development to prevent the earth environmental pollution, allowing re-utilization of resources.

In order to achieve the aforementioned objectives, the present invention provides a method of producing a magnetic toner according to claim 15, said toner comprising at least a binder resin, magnetic materials and additives.

The invention also provides an electrophotographic system as claimed in claim 16 using the improved magnetic toner. The present invention also provides the electrophotographic method as claimed in claim 17 using the improved magnetic toner comprises.

The magnetic toner of the invention according to claim 1 is characterized in that dielectric loss of the magnetic toner is 3.5 × 10⁻³ or less. The surface treatment is implemented by the surface treatment apparatus as claimed in claim 10.

The method of the invention, when applied, allows improvement in production efficiency by virtue of its continuous fashion. Also, since the surface treatment is carried out in a state of the toner dispersed, it is unlikely that toner particles will be fused with one another, thus preventing occurrence of rough particles. Also, the system involved is very simple and compact in construction. Other advantages include elimination of rise in wall temperature of the system housing, high yield of products, and unlikeliness of dust explosion by virtue of its open type of the system. There will be no agglomeration of toner particles one another due to instantaneous hot air treatment, which allows uniform treatment of toner particles as a whole. Bevels of toner particles that have developed over pulverization are completely removed so that the toner is sphered, improving the fluidity of the toner to a leap.

### BRIEF DESCRIPTION OF THE DRAWINGS

These and other objects and features of the present invention will become apparent from the following description taken in conjunction with the preferred embodiment thereof with reference to the accompanying drawings, in which:
Fig. 1 is a schematic view of the magnetic toner according to the present invention;
Fig. 2 is a picture of the overall surface of the magnetic toner according to the present invention observed by a scanning electron microscope;
Fig. 3 is a picture of local surface of the magnetic toner according to the present invention observed by a scanning electron microscope;
Fig. 4 is a schematic view showing the main part of the surface treatment apparatus for the magnetic toner according to an embodiment of the invention;
Fig. 5 is a schematic view showing the main part of an electrophotographic apparatus to which the electrophotographic method according to an embodiment of the present invention is applied;
Fig. 6 is a schematic view showing the main part of an electrophotographic apparatus to which the electrophotographic method according to an embodiment of the present invention is applied;
Fig. 7 is a picture of the overall surface of a magnetic toner of the prior art observed by a scanning electron microscope;
Fig. 8 is a picture of local surface of a prior-art magnetic toner observed by a scanning electron microscope;
Fig. 9 is a picture of the magnetic toner according to the present invention taken by a scanning electron microscope, showing an observational picture of the adhesion state of silicon oxide in an initial period;
Fig. 10 is a picture of the magnetic toner according to the present invention taken by a scanning electron microscope, showing an observational picture of the adhesion state of silicon oxide after a 10,000 sheet long-time copying test;
Fig. 11 is a picture of a prior-art magnetic toner taken by a scanning electron microscope, showing the adhesion state of silicon oxide in an initial period; and
Fig. 12 is a picture of a prior-art magnetic toner taken by a scanning electron microscope, showing an observational picture of the adhesion state of silicon oxide after a 10,000 sheet long-time copying test.

### DETAILED DESCRIPTION OF THE PREFERRED EMBODIMENTS

The present invention is described hereinbelow in more detail in connection with the attached drawings.

According to the electrophotographic system of the present invention, an electrostatic latent image is formed on an electrostatic latent image retaining member which contains a stationary magnet, and then the toner for the latent image is sprayed to the electrostatic latent image retaining member having an electrostatic latent image formed thereon, so that the toner magnetically adheres thereon is supported and transferred up to an electrode roller, where the toner on the electrostatic latent image retaining member corresponding to non-image areas is removed by electrostatic force and magnetic force by applying an AC bias power to the electrode roller.

In more detail, the electrophotographic system of the present invention utilizes a cascade development method in which a magnet is provided inside the electrostatic latent image retaining member and an AC voltage is applied to the electrode roller, thus allowing the system to be reduced in size and improved in performance.

In this method of the invention, when the toner is first sprayed onto the electrostatic latent image retaining member, the development of the image has almost been completed. The electrode roller portion allows the toner to circulate within a toner sump while it recovers the toner corresponding to non-image areas of the electrostatic latent image. In other words, it is the electrostatic latent image retaining member that supports and transfers the toner from the toner sump to the development section. The electrode roller is opposed to the electrostatic latent image retaining member by its bare face which supports no toner layer. The electrode roller and the electrostatic latent image retaining member rotate in opposite directions with each other.

The magnetic toner for use in the system of the present invention is preferably an insulating mono-component toner. Use of a mono-component toner eliminates the processes of mixing of carrier and toner as well as toner concentration control, which would be involved in the two-component development, thus allowing the system construction to be simplified.

In the electrophotographic method of the present invention, the toner is once adhered to the entire surface of the electrostatic latent image retaining member, and then removing the toner corresponding to non-image areas by electrostatic force and magnetic force by the electrode roller. Thus, in this method the resulting image quality depends largely upon the charging characteristic and fluidity of the toner.

The magnetic toner according to the present invention is produced using known techniques. The toner is subjected to mixing, kneading, pulverization, additive treatment, and as required, classification.

In the mixing process, a binder resin, magnetic material, and additives such as charge control agent, detachant, and pigment to be added as required are uniformly dispersed by a mixer or the like having agitators, which process is implemented by known techniques.

In the kneading process, the mixed material is heated and internal additives are dispersed into the binder resin by shear force. The kneading process can be carried out by a known heating kneader. The heating kneader may be either a three-roll type, single-shaft screw type, two-shaft screw type, Banbury mixer type, and the like in which the material to be kneaded is kneaded by heating and applying a shear force.

Agglomerations obtained by the kneading process are roughly pulverized by a cutter mill or the like. The product is more finely pulverized by a jet mill or the like. Further as required, in the classification process, fine particles are cut by a dispersion separator so that a desired particle size distribution can be obtained. It is to be noted that mechanical type of pulverization and classification may also be used in the above process. For example, it may be a method in which the toner is thrown into the minute void between a fixed stator and a rotating roller, where it is pulverized. Also, the classification may alternatively be carried out by classification by centrifugal force derived from the rotating rotor. The classification in either case is a known process.

According to the method of the present invention, the resultant magnetic toner is subjected to surface treatment by applying hot air to the toner that has been pulverized and, as required, classified. In more detail, the toner is dispersion-sprayed from a dispersion nozzle serving as a dispersion spraying means by compressed air, and then hot air heated by a heater serving as a hot-air generation means is radiated to the resulting dispersed and sprayed toner, thus accomplishing the surface treatment.

One case of a conventional practice is to render the surface treatment by heat, whereas in the conventional method the toner is fed into circulating hot air flows for heat treatment, which would easily result in agglomeration among toner particles, such that the toner surface could not be treated into a uniform configuration. Besides in the conventional method of the surface treatment by heat, it would be also likely that dust explosion may occur, due to the hermetically closed system. Furthermore, in the conventional method, the toner is sphered by mechanical impacts, there would occur fusions of toner particles onto the rotating shaft or noise, vibrations, and the like due to presence of a rotating body.

The method of the invention allows improvement in production efficiency by virtue of its continuous fashion. Also, since the surface treatment is carried out in a state of the toner dispersed, it is unlikely that toner particles will be fused with one another, preventing occurrence of rough particles. Also, the system involved is very simple and compact in construction. Other advantages include elimination of rise in wall temperature of the system housing, high yield of products, and unlikeliness of dust explosion by virtue of the open type of the system. There will be no agglomeration of toner particles one another due to instantaneous hot air treatment, which allows uniform treatment of toner as a whole. Bevels of toner particles that have developed over pulverization are completely removed so that the toner is sphered, improving the fluidity of the toner to a leap.

The magnetic toner according to the present invention is subjected to surface treatment by dispersing and feeding the pulverized toner particles into hot air flows. By this treatment, the surface of the binder resin of the toner particles is melted so that the magnetic material exposed on the surface of the toner particles are coated with the binder resin, while the toner particles can be sphered simultaneously and instantaneously.

As a method of quantitative evaluation of spherality of a toner, the spherality can be obtained in quantity according to values of specific surface areas in a BET method for measuring a general nitrogen adhesion amount. The specific surface area is influenced by a particle diameter, specific gravity and feature of the surface of the toner. In order to obtain the best mode of the fluidity, it is preferable to use a toner having a specific surface area of 0.4 to 4.0 m²/g under a condition of having a volume mean particle diameter of 6 to 12 µm and a magnetic material adding amount of 20 to 60 % by weight. In the present embodiment, the quantitative evaluation is carried out using "Flow Sorb II 2300" made by Shimazu Seisakusho Co., Ltd..

In order to effectively perform the surface treatment with uniformity suppressing agglomeration of the toner, it is required to suitably adjust the temperature, air amount and air pressure in balance when in the process of the surface treatment.

The compression air pressure is set 5000 to 30 000 kg/m² for feeding the toner from a toner supply source to the inlet of the dispersion spraying means, the hot air flow amount generated by the hot air generating means is preferably set 0.1 to 2.0 Nm³/min, the pressure of the hot air 15 000 to 50 000 kg/m², and the temperature of the hot air is set in the range of 100 to 600°C. Further, it is preferable that the caliber of the opening portion of the toner spray means is made smaller than that of a toner transporting pipe 32 (see Fig. 4).

Furthermore, by providing a metal mesh 30 having its mesh open value of 30 to 200 µm at the opening portion of the toner spray means, the toner dispersion can be effectively carried out suppressing the agglomeration of the toner.

The magnetic toner according to the present invention is subjected to additive treatment in which additives are added to toner fine particles which have been obtained through the surface treatment. The additive treatment is implemented by a known agitation with a mixer or the like.

When charge amount of a toner is lowered, the toner will be weakened in image force with respect to the electrostatic latent image retaining member, such that the toner adhering to the electrostatic latent image retaining member will be easily removed by magnetic force with the result of lowered image density. Besides, there will occur larger amounts of toner scattering around characters. It has been found that the clearness of the resulting images are lowered for these reasons.

The magnetic toner according to the present invention is capable of covering magnetic materials exposed on the toner surface with a binder resin, so that the toner can be charged with large amounts of charges. Thus, a high image density can be obtained, free from toner scattering around characters, which allows clear images to be obtained.

Further, dielectric loss of the magnetic toner according to the present invention is 3.5 × 10⁻³ or less. Dielectric loss of 3.5 × 10⁻³ or less results in a small amount of magnetic material that is exposed on the magnetic toner surface, where increased surface resistance of the magnetic toner serves to suppress the charges obtained through triboelectrification from leaking. Thus, a magnetic toner which is kept charged with a large amount of charges can be offered.

The dielectric loss was measured in such a manner that the magnetic toner was molded into 12 mm diameter pellets under a pressure of 100 kg/cm² and measured at a 1 kHz frequency with an LCR meter.

Lower fluidity of the toner would cause the toner on the non-image area to intensely adhere to the electrostatic latent image retaining member, so that it cannot be removed, which causes background fogs and therefore deterioration of the resulting image. Further, it has also been found that non-uniformities would occur at solid black image areas. If the fluidity of toner is increased by increasing the amount of the additive silicon oxide, the toner is decreased in non-electrostatic adhesion force to the electrostatic latent image retaining member, with decreased background fogs and increased image density, facilitated solution of non-uniformities in solid black image areas. However, there yet occur problems such as filming of silicon oxide to the electrostatic latent image retaining member and white dots of silicon oxide agglomerations adhering to the solid black image areas.

The electrophotographic method proposed in the present invention has such an arrangement that, to make the toner adhere to the entire photoconductor in the development process, the toner and the photoconductor are in contact with each other over a longer period, compared with the conventional mono-component development. On this account, use of a magnetic toner in which the magnetic material is exposed on the toner surface is likely to incur damage on the photoconductor surface. Besides, if a large amount of the additive, silicon oxide, is added to enhance the fluidity of the toner, suspended particles of silicon oxide will be generated, so that the filming of the toner on the photoconductor tends to occur.

However, the magnetic toner of the present invention is capable of imparting high fluidity to the toner by a minimum of hydrophobic-treated silicon oxide through surface treatment. Besides, since the toner has been sphered, silicon oxide can adhere uniformly to the toner in the additive treatment, so that far less amount of suspended particles of silicon oxide will result as compared with the conventional toner that is not sphered. For this reason, there will never occur flaws of the photoconductor or filming due to the suspended particles of silicon oxide. Also, high image quality can be obtained, free from background fogging. Moreover, since the magnetic material is covered with the binder resin, there will be no damage to the photoconductor surface due to the magnetic material. In the magnetic toner of the present embodiment, the additives are preferably of hydrophobic silicon oxide having a specific surface area in a range of 50 to 300 m²/g.

The adding amount of additives is preferably 0.1 to 5.0 parts by weight relative to 100 parts by weight of the magnetic toner. To prevent agglomeration among the toner particles, adding amounts of 0.1 or more part by weight is needed, while 5.0 or more parts by weight would cause silicon oxide to scatter. Although hydrophobic silicon oxide is used as the additive in the present invention, yet other known additives may also be used such as of inorganic fine particles or organic fine particles. It is preferable to use organic fine particles having a volume mean particle diameter of at least 0.01 to 5 µm as the additives.

Further, the electrophotographic system proposed in the present invention has an arrangement of recycling after-transfer toner in development. After-transfer toner is swept off the photoconductive drum by a cleaning blade or the like, resulting in residual toner. In this processing, the toner undergoes a strong stress. In this case, a similar stress is involved if the cleaning method adopts a rigid-body roller, furbrush roller, or the like as well as the blade. In order to provide stable image quality even if the residual toner is recycled, it is necessary for the residual toner to be maintained with large charge amount and high fluidity.

The magnetic toner according to the present invention, which is subjected to sphering treatment, is capable of offering high fluidity. Further, the toner is subject to less decrease in fluidity to the stress which the toner is received from within the developing unit or from the cleaning blade, so that the toner is stable to a great extent.

The toner has proved to have a significant difference in the stability of fluidity from the conventional toner that has not been subjected to surface treatment. From observing the adhesion state of silicon oxide of the residual toner, it was found that the conventional toner has silicon oxide buried in the toner, a great change from the initial state. Conversely, the magnetic toner of the invention was observed to remain almost unchanged in the adhesion state of silicon oxide from the initial state. This may be attributed to the fact that high fluidity helps avoid any stress.

Furthermore, in the present invention, the magnetic toner may be subjected to surface treatment after subjected to the additive treatment to fix the silicon oxide. One of the reasons why the characteristic of toner is changed partially because the adhesion state of the silicon oxide is varied due to the stress. The variation causes the change of the fluidity and charge property. Moreover, the filming to the photoconductor is greatly influenced by the floating silicon oxide particles.

Therefore, the adhesion state of the silicon oxide can be made stable by fixing the silicon oxide, preventing occurrence of filming to the photoconductor.

Furthermore, in the conventional method, organic fine particles are added for improving the cleaning performance. However, simply by adding such organic particles, no satisfactory effect can be obtained. None the less, when there is a part insufficiently added with the particles, the floating particles are agglomerated to cause white lines or black lines on the image undesirably.

In the present invention, the floating particles of silicon oxide are fixed in the process of the surface treatment, thereby suppressing occurrence of agglomeration of the particles, resulting in effective cleaning.

As the organic fine particles, there may be used known materials such as acrylic resin, styrene resin, silicon resin groups and polytetrafluoroethylene, where the volume average diameter of the particles is preferably 0.01 to 5 µm.

In other words, the surface treated toner will undergo less change in the adhesion state of silicon oxide in recycling use, thus able to maintain the high fluidity.

The magnetic toner according to the present invention comprises at least a binder resin, a magnetic material, and an additive.

The binder resin of the magnetic toner according to the present invention is of a vinyl copolymer in which vinyl monomers have been polymerized or copolymerized. Examples of the monomer styrene constituting the binder resin include monocarboxylic acids having double bonds and their substitutes of styrene such as styrene, α-methyl styrene, and P-chlorostyrene, and their substitutes; alkylester acrylate such as acrylic acid, methyl acrylate, ethyl acrylate, butyl acrylate, dodecyl acrylate, octyl acrylate, isobutyl acrylate, and hexyl acrylate; alkylester methacrylate such as methyl methacrylate, ethyl methacrylate, butyl methacrylate, octyl methacrylate, isobutyl methacrylate, dodecyl methacrylate, and hexyl methacrylate.

As the method of producing these copolymers there are available known copolymerization methods such as bulk polymerization, solution polymerization, suspension polymerization, and emulsion polymerization.

The copolymer used for the magnetic toner according to the present invention preferably contains 50 to 95% by weight of styrenic components. Less than 50% by weight of styrene causes the toner to be deteriorated in melt characteristic, insufficient fixability, and worsened pulverizability.

Whereas the magnetic toner according to the present invention has a binder resin like those above mentioned as a main component, other known polymers or copolymers may also be used in addition to such main component, as required. Examples of those are polyester resins, epoxy resins, and polyurethane resins.

The magnetic toner according to the present invention has other known additives added thereto as required. Preferable materials of the additives are known inorganic fine particle materials such as hydrophobic silicon oxide, titanium oxide, aluminum oxide, and zirconium oxide. Whereas hydrophobic silicon oxide, for example, can be obtained in such a manner that hydrophilic silicon oxide obtained by treating silicon tetra-chloride is subjected to further surface treatment, there are available such known treating agents, to which negative-chargeability and hydrophobic property have been taken into consideration, as dimethyl-dichloro-silane, hexamethylenedisilazane, and dimethyl-siloxane, which are all effective to the hydrophobic property and negative-chargeability.

The magnetic toner according to the present invention has appropriate pigments or dyes blended therewith, as required, for the purpose of coloring and charge control. As such pigments or dyes, there are carbon black, iron black, graphite, nigrosine, metal complexes of azo-dyes, phthalocyanine blue, Du Pont oil red, aniline blue, benzine yellow, rose bengal, and their mixtures, where the blending amount of them depends on the amount of charging and coloring.

The magnetic toner according to the present invention has a detachant further blended therewith as required. The magnetic toner may have other types of additives further blended therewith as required. For example, they are abrasives such as tin oxide, strontium titanate, and tungsten carbide. There may also be added, as required, fine particles of organic material as fluidity aid, charging aid, cleaning aid, and the like.

Still further, the magnetic toner according to the present invention has a magnetic material blended therewith. As the magnetic powder, there are available metal powders of iron, manganese, nickel, cobalt, and the like, and ferrites of iron, manganese, nickel, cobalt, zinc, and the like. Mean particle size of the powder is preferably 1 µm or less, more preferably 0.6 µm or less. The adding amount is preferably 20 to 60% by weight. Less than 20% by weight of adding amount likely causes toner scattering to increase, while more than 60% by weight of addition likely causes the toner charge amount to decrease, which leads to deterioration of image quality.

By using the magnetic toner of large charge amount and high fluidity obtained through surface treatment with the above-described arrangement, it is possible to offer high quality of images with high density and low background fogging by a development method which allows the system to be further reduced in size, simplified in construction, and lowered in cost. Furthermore, since the residual toner to be recycled can maintain high fluidity and high chargeability, it being possible to recycle the residual toner, a magnetic toner can be provided which eliminates the need of disposal thereof and which allows prevention of earth environmental pollution and re-utilization of resources through recycling of the toner.

Hereinbelow, a magnetic toner according to an embodiment of the present invention is described with reference to the accompanying drawings. The present invention is, however, not limited to these examples.

### First Embodiment

Table 1 shows an example of the material composition of magnetic toner A according to the present invention.

**Table 1:**

| | | |
|---|---|---|
| Binder resin | Styrene-butyl acrylate copolymer resin (monomer ratio: 82/18) | 62.5% |
| | Melt viscosity at 135°C: 1 × 10⁵ (poise) | |
| | Melt viscosity at 145°C: 2 × 10⁴ (poise) | |
| Magnetic material | Magnetite | 35% |
| Charge control agent | Cr-metallized azo-dye | 1% |
| Detachant | Polypropylene | 1.5% |
| Additive | Hydrophobic silicon oxide | 1.0 part |

A production method of the magnetic toner according to the present invention is described below. The mixture as shown in Table 1 is mixed by a Henschel mixer FM20B (made by Mitsui Miike Engineering Co.). The mixture is heated and kneaded by a two-shaft kneading extruder PCM30 (made by Ikegai Co.). The kneaded product is fine pulverized by a jet mill IDS2 (made by Nihon Pneumatic MFG. Co.). The pulverized fine particles are cut by a dispersion separator DS2 (made by Nihon Pneumatic MFG. Co.). Through these steps, particles with a 8 µm mean particle size were obtained. Then the particles were subjected to surface treatment at a hot air temperature of 300°C by the surface treatment apparatus as shown in Fig. 4. Thereafter, hydrophobic silicon oxide of inorganic fine particles was mixed with the surface treated particles for additive treatment by the Henschel mixer FM20B (made by Mitsui Miike Engineering Co.).

An embodiment of the surface treatment apparatus for the magnetic toner according to the present invention as shown in Fig. 4 is now described.

Referring to Fig. 4, a magnetic toner 22 is thrown from a measuring feeder 21 and transferred to dispersion nozzles 24, which are means for dispersing the magnetic toner, by a compressed air 23, from which nozzles the magnetic toner is sprayed in the approximately 45 degrees direction. The compressed air 23 is fed by a compressed air supply unit (31) for supplying the compressed air which contains the magnetic toner dispersed. Furthermore, by providing a metal mesh 30 having its mesh open value of 30 to 200 µm at the opening portions of the toner spray nozzles, the toner dispersion can be effectively carried out suppressing the agglomeration of the toner.

In the present invention, the dispersion nozzles 24 were provided at least two in number at right-to-left symmetrical positions in the figure. This is because a plurality of nozzles allow the magnetic toner to be treated more uniformly when sprayed therefrom. For radiation of hot air to the magnetic toner 22 sprayed from the dispersion nozzles 24, hot air 26 is generated from a hot air generation device 25. In the present invention, a heater is used for the hot air generation device. The device is not limitative but may be whatever can generate hot air. The magnetic toner 22 disperses and passes with the hot air 26 to be subjected to surface treatment. The surface treated magnetic toner is taken into a hood 28, collected in a cyclone (not shown) located as pointed by arrow 29.

Fig. 1 shows a schematic constitution of a magnetic toner according to the present invention, where reference numeral 1 denotes a binder resin, 2 denotes a magnetic material particle, 3 denotes a charge control agent, 4 denotes a detachant, and 5 denotes hydrophobic silicon oxide.

Fig. 2 shows an observational image of the overall surface of the magnetic toner according to the present invention taken by a scanning electron microscope, where the magnifying power is 3,000.

Fig. 3 shows an observational image of a local surface of the magnetic toner according to the present invention taken by a scanning electron microscope, where the magnifying power is 30,000.

As shown in Fig. 2, the overall configuration of the toner is sphered. In Fig. 3, where it is further enlarged, the image of the magnetic material surface is blurred, which shows that the magnetic material is coated. White dots in Figs. 2 and 3 represent magnetic material particles.

Physical property values of the magnetic toner A according to the present invention are listed in Table 2. Hot air temperature is selected as a parameter for surface treatment. As a comparative example, physical property values of magnetic toner B that has not been subjected to surface treatment are also listed in the table. Fluidity is defined by apparent density. The measurement was carried out by using a powder tester made by Hosokawa Micron Co. Charge amount was measured by the blowoff method. As measuring conditions, toners were mixed with non-coated ferrite carriers at a toner concentration of 10%, put into a 100 ml polyethylene bottle, and agitated at 60 rpm for 10 min.

**Table 2:**

| Toner | Hot air temperature (°C) | Apparent density (g/cc) | Charge amount (µC/g) | Dielectric loss (× 10⁻³) |
|---|---|---|---|---|
| Toner A | 300 | 0.61 | -31.0 | 2.8 |
| Toner A | 350 | 0.64 | -34.0 | 2.4 |
| Toner A | 400 | 0.655 | -36.5 | 2.2 |
| Toner B | - | 0.43 | -20.5 | 5.1 |

It is understood that magnetic toner A clearly shows high fluidity, high chargeability, and low dielectric loss.

### Second Embodiment

Fig. 5 shows an example of the electrophotographic system according to the present invention. In this development system, there is employed a mono-component magnetic toner. Reference numeral 101 denotes an organic photoconductive drum in which phtharocyanine has been dispersed in polyester binder resin; 102 denotes a magnet fixed coaxial with the photoconductor 101; 103 denotes a corona charger for negatively charging the photoconductor; 104 denotes a grid electrode for controlling the charging voltage of the photoconductor. A laser beam 105 is applied to the surface of the photoconductive drum 101 as a signal light. Reference numeral 106 denotes a toner sump for storing a magnetic mono-component toner 107. Reference numeral 108 denotes a non-magnetic electrode roller set with a gap open to the photoconductor 101; 109 denotes a magnet located inside the non-magnetic electrode roller 108; 110 denotes an AC high-voltage power supply for applying AC voltage to the electrode roller 108; 117 denotes a negative DC bias power supply; 111 denotes a scraper made of polyester film for sweeping off the toner on the electrode roller; and 112 denotes a transfer corona charger for transferring the toner image formed on the photoconductor onto a copying sheet 118 such as paper to be visualized. Further, 113 denotes a damper for smoothing the flow of the toner within the toner sump 106 and preventing the toner from being crushed by dead weight, which may cause blinding between the photoconductor 101 and the electrode roller 108.

The magnetic flux density on the surface of the photoconductor 101 is set around 600 Gs. The magnetic force inside the electrode roller 108 is more strengthened, thereby improving the transportability of the toner. The pole angle θ of the magnet 102 as shown in the figure was set to 15 degrees. The photoconductor 101, having a diameter of 30 mm, was rotated at a circumferential velocity of 60 mm/s in the clockwise direction indicated by an arrow **Ra** in the figure. The electrode roller 108, having a diameter of 16 mm, was rotated at a circumferential velocity of 40 mm/s in the clockwise direction reverse to the forward direction of the photoconductor as indicated by an arrow **Rb** in the figure. The gap between the photoconductor 101 and the electrode roller 108 was defined by a distance of 300 µm.

The photoconductor 101 was charged to -500 V by the corona charger 103, where applied voltage was -4.5 kV, Grid (104) voltage was -500 V. A laser beam 105 was applied to the photoconductor 101 to form an electrostatic latent image thereon. In this process, the exposure voltage of the photoconductor was -90 V. The toner 107 was made to adhere onto the surface of the photoconductor 101 in the toner sump 106 by the magnet 102. Then the toner adhered portion of the photoconductor 101 was passed by in front of the electrode roller 108. While uncharged areas of the photoconductor 101 passed by, a 750 VO-p (peak-to-peak: 1.5 kV) AC voltage (frequency: 1 kHz) on which a DC voltage of 0 V was superimposed was applied to the electrode roller 108 by the AC high-voltage power supply 110. Thereafter, while the areas of the photoconductor 101 that had been charged to -500 V to have an electrostatic latent image written therein was passed by, a 750 V0-p (peak-to-peak: 1.5 kV) AC voltage (frequency: 1 kHz) on which a -350 V DC voltage was superimposed was applied to the electrode roller 108 by the AC high-voltage power supply 110. As a result, the toner adhering to the charged portions of the photoconductor 101 was recovered by the electrode roller 108, with the result that there remained a negative-positive inverted toner image of only image areas on the photoconductor 101. The toner adhering to the electrode roller 108 that would rotate in the direction of arrow Rb was swept off by the scraper 111, being returned into the toner sump 106 and used for formation of the succeeding image. The toner image obtained on the photoconductor 101 in this way is then transferred onto paper 118 by the transfer corona charger 112, and subsequently thermally fixed by a fixing unit (not shown), thus producing a copied image.

By using the electrophotographic system as shown in Fig. 5, a copying test was conducted with the magnetic toner A of the first embodiment that had been surface treated. Image density was measured by a reflection density meter (made by Macbeth Co.), followed by evaluation. As a result, an image was obtained which was of extremely high resolution and high image quality, free from any disorder of horizontal lines or toner scattering, uniform in solid black, and in which 16 lines/mm image lines with a density of 1.4 could be reproduced. A high-density image with an image density of 1.4 or more could be obtained. There developed no background fogs at non-image areas.

### Third Embodiment

Fig. 6 shows another embodiment of the electrophotographic system according to the present invention. The third embodiment is different from the second embodiment in the fact that the electrophotographic system is further provided with a residual toner recycle process means. Reference numeral 114 denotes a cleaning blade for sweeping off the residual toner remaining after transfer, 115 denotes a transport tube for transferring the residual toner to the toner sump 106, and 116 denotes a cleaning box for temporarily storing the residual toner. The rest of the arrangement is the same as the second embodiment shown in Fig. 5.

By using the electrophotographic system as shown in Fig. 6, a copying test was conducted with the magnetic toner A of the present invention, as shown in the first Embodiment, that had been surface treated. Image density was measured by a reflection density meter (made by Macbeth Co.), followed by evaluation. As a result, an image was obtained which was of extremely high resolution and high image quality, free from any disorder of horizontal lines or toner scattering, uniform in solid black, and in which 16 lines/mm image lines with a density of 1.4 could be reproduced. A high-density image with an image density of 1.4 or more could be obtained. There developed no background fog at non-image areas.

Further, with the residual toner recycled, a long-period copying test was conducted with 10,000 sheets of copy. After 10,000 sheets of copy, it was shown that the toner was free from deterioration in fluidity, high charge amount was maintained, and that there occurred no filming on the photoconductor. High-density, low-background-fogging copied images could be obtained, comparable to the initial images. The toner also exhibited a satisfactory recyclability.

Fig. 9 is a picture of a magnetic toner A according to the present invention observed by a scanning electron microscope, showing a picture of the adhesion state of silicon oxide in the initial period.

Fig. 10 is a picture of the magnetic toner A observed by a scanning electron microscope, showing a picture of the adhesion state of silicon oxide after a long-period copying test of 10,000 sheets of copy, where the magnifying power was 30,000. Large white dots represent magnetic material particles and small fine dots represent silicon oxide particles. Silicon oxide particles could be viewed clearly both in the initial period and after the copying test, showing that the particles maintain their uniform adhesion state.

Table 3 lists the toner fluidity and image density both in the initial period and after the 10,000 sheet copying test.

**Table 3:**

| Toner | Apparent density | | Image density | |
|---|---|---|---|---|
| | Initial | After copying test | Initial | After long-period test |
| Toner A | 0.61 | 0.60 | 1.42 | 1.41 |
| Toner B | 0.43 | 0.34 | 1.10 | 0.85 |

It is understood that the toner showed less variation in both fluidity and image density, exhibiting stable characteristics.

### Comparative Example 1

Magnetic toner B of Comparative Example 1 is similar in material composition and production method to Embodiment 1 except that it is not subjected to surface treatment.

Fig. 7 shows an observational image of the overall surface of the prior-art magnetic toner B taken by a scanning electron microscope. It can be clearly seen that the toner configuration is of variable pattern.

Fig. 8 shows an observational image of local surface of the magnetic toner B taken by a scanning electron microscope. It can be clearly seen that magnetic material particles are exposed in the surface.

Physical property values of the magnetic toner B as shown in Table 2 also show that the toner has lower fluidity, lower charge amount, and higher dielectric loss, as compared with magnetic toner A.

If the hot air temperature is 50°C, the resulting physical properties of the toner are equivalent to those of the toner that has not been surface treated.

Also, if the hot air temperature is 650°C, agglomerations were developed to a great amount among toner particles. Besides, other additives are beginning to show thermal damage. Power consumption is too much to allow practical use of the toner.

### Comparative Example 2

By using the magnetic toner B that is not subjected to surface treatment as shown in Comparative Example 1, the copying test was conducted by the electrophotographic method presented in Embodiment 2. The resulting image density was no higher than 1.1, there was a large amount of background fogs at non-image areas, so that no practical image could not be obtained.

### Comparative Example 3

By using the magnetic toner B that is not subjected to surface treatment as shown in Comparative Example 1, the copying test was conducted by the electrophotographic method presented in Embodiment 3. The resulting image density was no higher than 1.1, there was a large amount of background fogs at non-image areas, so that no practical image could not be obtained. In the long-period copying test, there developed pronounced deterioration in the toner fluidity, lowering of image density, and increase in background fogs at non-image areas.

Fig. 11 is an observational image by a scanning electron microscope, showing the adhesion state of initial silicon oxide.

Fig. 12 is an observational image by a scanning electron microscope, showing the adhesion state of silicon oxide after the 10,000 sheet long-period copying test. The magnifying power was 30,000. In the initial state, particles of silicon oxide can be seen, but they adhere in their partially agglomerated state, which is a less uniform adhesion state as compared with Example 3. After the copying test, silicon oxide particles cannot be seen, showing that they are buried in the toner. This accounts for the reduction in fluidity. Table 3 lists the fluidity and image density of the toner both in the initial period and after the 10,000 sheet copying test. It is understood that both fluidity and image density of the toner are deteriorated.

Although the present invention has been fully described by way of example with reference to the accompanying drawings, it is to be noted here that various changes and modifications will be apparent to those skilled in the art. Therefore, unless otherwise such changes and modifications depart from the scope of the present invention as defined by the appended claims, they should be construed as included therein.

## Claims

1. An electrophotographic magnetic toner composed of toner particles for use in an electrophotographic system capable of recycling residual toner for developing an image,
wherein each toner particle comprises at least a binder resin (1), a magnetic powder material (2) and additives (3, 4) kneaded and dispersed by thermal melting,
each toner particle has a spherical surface, and each fine particle (2) of said magnetic powder material is coated with said binder resin (1), and wherein
the magnetic toner has a volume mean particle diameter in the range of 6 to 12 µm and a specific surface area in the range of 0.4 to 4.0 m²/g,
**characterized in that**
the magnetic toner has a dielectric loss of at most 3.5 × 10⁻³.

2. The magnetic toner of claim 1, wherein said magnetic toner is a mono-component toner.

3. The magnetic toner of claim 1 or 2, wherein said additives are hydrophobic silicon oxide (5) having a specific surface area in the range of 50 to 300 m²/g.

4. The magnetic toner of claim 1 or 2, wherein said additives are organic fine particles each having a volume mean particle diameter of at least 0.01 to 5 µm.

5. The magnetic toner of one of claims 1 to 4, wherein the adding amount of said additives is 0.1 to 5.0 parts by weight relative to 100 parts by weight of the magnetic toner.

6. The magnetic toner of anyone of the preceding claims, wherein said binder resin (1) of the magnetic toner is a vinyl copolymer in which vinyl monomers have been polymerized or copolymerized.

7. The magnetic toner of anyone of the preceding claims, wherein said magnetic toner comprises appropriate pigments or dyes blended therewith for the purpose of coloring and charge control.

8. The magnetic toner of anyone of the preceding claims, wherein said magnetic toner further comprises a detachant (4) blended therewith.

9. The magnetic toner of anyone of the preceding claims, wherein said magnetic toner comprises a magnetic powder material (2) blended therewith, and metal powder of any one of iron, manganese, nickel, cobalt, and zinc is used as the magnetic powder, and the mean particle size of the magnetic powder material is at most 1 µm while the adding amount thereof is 20 to 60 % by weight.

10. An apparatus for implementing the surface treatment of the electrophotographic magnetic toner according to anyone of the preceding claims with uniformily suppressing agglomeration of the toner, the apparatus comprising:
toner supply means (21) for supplying the magnetic toner (22) at a constant feeding rate;
spraying means (24) for dispersion-spraying the magnetic toner;
compressed air supply means (31) for supplying compressed air (23) containing the magnetic toner (22) to said spraying means (24) through a toner transporting pipe (32);
hot air generation means (25) for applying hot air (26) to the magnetic toner (22) sprayed from said spraying means (24); and
toner recovery means (28, 29) for recovering the magnetic toner according to claims 1-9
dispersion-sprayed in the hot air (26),
wherein the caliber of the opening portion of the toner spray means (24) is smaller than that of the toner transporting pipe (32).

11. The apparatus of claim 10, wherein the compression air pressure is set to be 5 000 to 30 000 kg/m² for feeding the toner from said toner supply means (21) to the inlet of the spraying means (24), the pressure of the hot air is set to be 15 000 to 50 000 kg/m², and the temperature of the hot air is set to be in the range of 100 to 600 °C.

12. The apparatus of claim 10 or 11, further comprising a metal mesh (30) having an aperture value of 30 to 200 µm at the opening portion of said spraying means (24) for suppressing the agglomeration of the toner.

13. The apparatus anyone of claims 10 to 12, wherein said toner spraying means comprises at least a pair of dispersion nozzles (24) with compressed air, from which nozzles (24) the magnetic toner is sprayed with compresses air (23) in the approximately 45 degrees direction.

14. The apparatus of claim 13, wherein the dispersion nozzles (24) are provided two in number at right-to-left symmetrical positions with respect to said hot air generation means (25).

15. A method for producing the electrophotographic magnetic toner according to anyone of claims 1 to 9, the method comprising the steps of:
kneading a binder resin (1), fine particles (2) of a magnetic material and additives (3, 4),
pulverizing the resulting kneaded materials,
classifying the pulverized material, and
effecting surface treatment of the classified material by hot air in its dispersed state to accomplish sphering of the magnetic toner,
**characterized in that**
the surface treatment is effected by melting the surface of the binder resin (1) such that each fine particle (2) of the magnetic material being exposed on the surface of the magnetic toner is coated with the binder resin (1) and the toner particles are sphered simultaneously and instantaneously, under the condition that the compression air pressure is set to be in the range of 5 000 to 30 000 kg/m², the pressure of the hot air in the range of 15 000 to 50 000 kg/m², and the temperature of the hot air in the range of 100 to 600 °C.

16. An electrophotographic system using the electrophotographic magnetic toner according to anyone of claims 1 to 9, the system comprising:
development means which comprises a rotatable electrostatic latent image retaining member (101) which contains a stationary magnet (102); toner sump means (106) which is opposed to a surface of the electrostatic latent image retaining member (101) to feed the magnetic toner by causing the stationary magnet (102) to suck the magnetic toner magnetically; and an electrode roller (108) which is located at a specified interval from the surface of the electrostatic latent image retaining member (101) and which contains a magnet (109) therein;
transfer means (112) for transferring the magnetic toner onto a transfer material (118) for visualisation of the electrostatic latent image formed on the electrostatic latent image retaining member (101);
cleaning means (114, 116) for removing the magnetic toner partially remaining after transfer on the electrostatic latent image retaining member (101) from the same; and
toner recycling means (115) for returning the magnetic toner that has been removed in the cleaning means (114, 116) again to the development process for the purpose of recycling;
wherein the toner adhering to the charged portions of said electrostatic latent image retaining menber (101) is recovered by the electrode roller (118), with the result that there remains on said electrostatic latent image retaining member (101) a negative-positive inverted toner image only with respect to the image areas.

17. An electrophotographic method using the electrophotographic magnetic toner according to anyone of claims 1 to 9, the method comprising the steps of
retaining an electrostatic latent image a latent image retaining member (101);
developing the retained electrostatic latent image to be visualized with the magnetic toner fed by causing the stationary magnet (102) to suck the toner magnetically;
transferring the developed image with the magnetic toner onto a transfer member (112);
cleaning the latent image retaining member (101) for removing the magnetic toner partially remaining after the transfer process; and
recycling the tone for returning the magnetic toner that has been removed in the cleaning precess again to the development process for the purpose of recycling.

## Patentansprüche

1. Elektrophotographischer Magnettoner, der sich aus Tonerpartikeln zusammensetzt und der für ein elektrophotographisches System verwendbar ist,
welches zum Wiedergewinnen von übrig gebliebenem Toner für die Entwicklung eines Bildes in der Lage ist,
wobei jeder Tonerpartikel zumindest ein Bindeharz (1), ein magnetisches Pulvermaterial (2) und Zusätze (3, 4, 5) enthält, die geknetet und durch Warmschmelzen dispergiert werden,
wobei jeder Tonerpartikel eine kugelförmige Oberfläche aufweist,
wobei jeder Feinpartikel (2) des magnetischen Pulvermaterials mit dem Bindeharz (1) beschichtet ist, und
wobei der elektrophotographische Magnettoner einen mittleren Volumenpartikeldurchmesser im Bereich von 6 bis 12 µm und eine wirksame Oberfläche im Bereich von 0,4 bis 4,0 m²/g aufweist,
**dadurch gekennzeichnet**, daß der elektrophotographische Magnettoner einen Dielektrizitätsverlust von höchstens 3,5 x 10⁻³ aufweist.

2. Magnettoner nach Anspruch 1,
bei dem der elektrophotographische Magnettoner ein Einkomponententoner ist.

3. Magnettoner nach Anspruch 1 oder 2,
bei dem die Zusätze wasserabweisendes Siliziumoxid (5) sind, das eine wirksame Oberfläche im Bereich von 50 bis 300 m²/g aufweist.

4. Magnettoner nach Anspruch 1 oder 2,
bei dem die Zusätze organische Feinpartikel sind, die jeweils einen mittleren Volumenpartikeldurchmesser von zumindestens 0,01 bis 5 µm besitzen.

5. Elektrophotographischer Magnettoner nach einem der Ansprüche 1 bis 4,
**dadurch gekennzeichnet**, daß die hinzugefügte Menge der Zusätze 0,1 bis 5,0 Gewichtsteile bezogen auf 100 Gewichtsteile des Magnettoners beträgt.

6. Magnettoner nach einem der vorstehenden Ansprüche,
bei dem das Bindeharz (1) des Magnettoners ein Vinylcopolymer ist, bei dem Vinylmonomere polymerisiert oder copolymerisiert worden sind.

7. Magnettoner nach einem der vorstehenden Ansprüche,
bei dem der Magnettoner geeignete Pigmente oder Farbe enthält, die zum Zwecke des Einfärbens und der Ladungssteuerung eingemischt werden.

8. Magnettoner nach einem der vorstehenden Ansprüche,
bei dem der Magnettoner weiterhin ein Ablösemittel (4) enthält, das mit ihm vermischt ist.

9. Magnettoner nach einem der vorstehenden Ansprüche,
bei dem der Magnettoner ein magnetisches Pulvermaterial (2) enthält, das mit ihm vermischt ist, bei dem metallisches Pulver aus einem der nachfolgenden Elemente: Eisen, Magnesium, Nickel, Kobalt und Zink als magnetisches Pulver verwendet wird und bei dem die mittlere Partikelgröße des magnetischen Pulvermaterials höchstens 1 µm beträgt, während die hinzugefügte Menge 20 bis 60 Gew.-% beträgt.

10. Vorrichtung zum Durchführen der Oberflächenbehandlung des elektrophotographischen Magnettoners nach einem der vorstehenden Ansprüche, bei der gleichförmig die Agglomeration des Toners unterdrückt wird und die enthält: Tonerzuführmittel (21) zum Zuführen des Magnettoners (22) mit einer konstanten Zuführgeschwindigkeit,
Sprühmittel (24) für ein Dispersionsprühen des Magnettoners,
Druckluft-Zuführmittel (31) zum Zuführen der den Magnettoner (22) enthaltenden Druckluft (23) zu den Sprühmitteln (24) über ein Tonertransportrohr (32),
Heißlufterzeugungsmittel (25) zum Beaufschlagen des von den Sprühmitteln (24) versprühten Magnettoners (22) mit heißer Luft (26), und
Tonerwiedergewinnungsmittel (28, 29) zum Wiedergewinnen des Magnettoners nach einem der Ansprüche 1 bis 9, der in der heißen Luft (26) dispersionsversprüht wird,
wobei das Kaliber des Öffnungsabschnittes des Tonersprühmittels (24) kleiner als das Kaliber des Tonertransportrohres (32) ist.

11. Vorrichtung nach Anspruch 10,
bei der der Druck der Druckluft auf 5.000 bis 30.000 kg/m² zum Zuführen des Toners aus dem Tonerzuführmittel (21) zu dem Einlaß des Sprühmittels (24) eingestellt wird, bei der der Druck der Heißluft auf 15.000 bis 50.000 kg/m² eingestellt wird und bei der die Temperatur der Heißluft auf einen Bereich von 100° C bis 600° C eingestellt wird.

12. Vorrichtung nach Anspruch 10 oder 11,
weiterhin enthaltend ein Metallnetz (30), das einen Öffnungswert von 30 bis 200 µm an dem Öffnungsabschnitt des Sprühmittels (24) zum Unterdrücken der Agglomeration des Toners aufweist.

13. Vorrichtung nach einem der Ansprüche 10 bis 12,
bei der das Tonersprühmittel zumindest ein Paar Dispersionsdüsen (24) mit Druckluft aufweist, wobei der Magnettoner mit Druckluft (23) in eine Richtung von annähernd 45° von den Düsen (24) aus versprüht wird.

14. Vorrichtung nach Anspruch 13,
bei der zwei Dispersionsdüsen rechts und links in symmetrischen Positionen mit Bezug auf die Heißluft-Erzeugungsmittel (25) angeordnet sind.

15. Verfahren zum Herstellen des elektrophotographischen Magnettoners nach einem der Ansprüche 1 bis 9, wobei das Verfahren die folgenden Schritte enthält:
Kneten eines Bindeharzes (1), von Feinpartikeln (2) eines magnetischen Materials und von Zusätzen (3, 4, 5),
Pulverisieren des sich ergebenden, gekneteten Materials,
Klassifizieren des pulverisierten Materials und
Ausführen einer Oberflächenbehandlung des klassifizierten Materials mittels heißer Luft in seinem dispergierten Zustand, um die Kugelbildung des Magnettoners auszuführen,
**dadurch gekennzeichnet**, daß die Oberflächenbehandlung durch Schmelzen der Oberfläche des Bindeharzes (1) in der Weise ausgeführt wird, daß jeder Feinpartikel (2) des magnetischen Materials, der auf der Oberfläche des Magnettoners vorhanden ist, mit dem Bindeharz (1) beschichtet wird und die Tonerpartikel gleichzeitig sowie unverzüglich unter der Bedingung in Kugelform gebracht werden, daß der Druck der Druckluft auf einen Bereich von 5.000 bis 30.000 kg/m², der Druck der Heißluft im Bereich von 1 5.000 bis 50.000 kg/m² und die Temperatur der Heißluft im Bereich von 100° C bis 600° C eingestellt wird.

16. Elektrophotographisches System, das den elektrophotographischen Magnettoner nach einem der Ansprüche 1 bis 9 verwendet und das enthält:
ein Entwicklungsmittel, das ein drehbares, elektrostatisches Latentbild-Halteelement (101) aufweist, welches einen stationären Magneten (102) enthält, ein Tonerauffangmittel (106), welches zu einer Oberfläche des elektrostatischen Latentbild-Halteelements (101) gegenüberliegend angeordnet ist, um den Magnettoner zuzuführen, in dem der stationäre Magnet (102) den Magnettoner magnetisch anzieht, und eine Elektrodenwalze (108), die in einem bestimmten Abstand von der Oberfläche des elektrostatischen Latentbild-Halteelements (101) angeordnet ist und die einen Magneten (109) aufnimmt,
Transfermittel (112) zum Übertragen des Magnettoners auf ein Transfermaterial (118) zum Sichtbarmachen des elektrostatischen Latentbilds, das auf dem elektrostatischen Latentbild-Halteelement (101) gebildet ist,
Reinigungsmittel (114, 116) zum Entfernen des Magnettoners von dem elektrostatischen Latentbild-Halteelements (101), der nach dem Übertragen auf diesem übrig bleibt, und
Tonerwiedergewinnungsmittel (115) zum Zurückführen des durch die Reinigungsmittel (114, 116) entfernten Magnettoners zu dem Entwicklungsvorgang zum Zwecke der Wiedergewinnung,
wobei der auf den aufgeladenen Abschnitten des elektrostatischen Latentbild-Halteelements (101) haftende Toner durch die Elektrodenwalze (118) mit dem Ergebnis zurückgeführt wird, daß auf dem elektrostatischen Latentbild-Halteelement (101) ein negativ-positiv umgekehrtes Tonerbild nur hinsichtlich der Bildbereiche übrig bleibt.

17. Elektrophotographisches Verfahren, welches den elektrophotographischen Magnettoner nach einem der Ansprüche 1 bis 9 verwendet und welches die folgenden Schritte enthält:
Halten eines elektrostatischen Latentbildes auf einem Latentbild-Halteelement (101),
Entwickeln des gehaltenen elektrostatischen und zu visualisierenden Latentbildes mit dem Magnettoner, der dadurch zugeführt wird, daß der stationäre Magnet (102) den Toner magnetisch anzieht,
Übertragen des mit dem Magnettoner entwickelten Bildes auf ein Transferelement (112),
Reinigen des Latentbild-Halteelements (101), um den Magnettoner zu entfernen, der teilweise nach dem Transfervorgang übrig bleibt, und
Wiedergewinnen des Toners zum Zurückführen des in dem Reinigungsprozeß entfernten Magnettoners zu dem Entwicklungsvorgang zum Zwecke des Wiedergewinnens.

## Revendications

1. Toner magnétique électrophotographique composé de particules de toner, destiné à être utilisé dans un dispositif électrophographique capable de recycler le toner résiduel pour le développement d'une image,
dans lequel chaque particule de toner comprend au moins une résine de liaison (1), une matière magnétique en poudre (2) et des additifs (3,4,5) malaxés et dispersés par fusion thermique.
chaque particule de toner a une surface sphérique, et
chaque particule fine (2) de la dite matière magnétique en poudre est revêtue de ladite résine de liaison (1), et dans lequel
le toner magnétique a un diamètre du volume de particule moyen dans la plage allant de 6 à 12 µm et une surface spécifique dans la plage allant de 0.4 à 4.0 m²/g,
caractérisé en ce que
le toner magnétique a une perte diélectrique au plus de 3.5 X 10⁻³.

2. Toner magnétique selon la revendication 1, dans lequel le dit toner magnétique est un toner à un composant.

3. Toner magnétique selon la revendication 1 ou 2, dans lequel lesdits additifs sont de l'oxyde de silicium hydrophobe (5) ayant une surface spécifique dans la plage allant de 50 à 300 m²/g.

4. Toner magnétique selon la revendication 1 ou 2, dans lequel les dits additifs sont des particules organiques fines ayant chacune un diamètre du volume de particule moyen d'au moins 0,01 à 5 µm.

5. Toner magnétique selon l'une des revendications 1 à 4, dans lequel la quantité additionnée desdits additifs va de 0,1 à 5,0 parties en poids par rapport aux 100 parties en poids du toner magnétique.

6. Toner magnétique selon l'une quelconque des revendications précédentes, dans lequel ladite résine de liaison (1) du toner magnétique est un copolymère de vinyle dans lequel des monomères de vinyle ont été polymérisés ou copolymérisés.

7. Toner magnétique selon l'une quelconque des revendications précédentes, dans lequel ledit toner magnétique comprend des pigments ou des teintures appropriées mélangés avec celui-ci dans le but de coloriage et de contrôle de charge.

8. Toner magnétique selon l'une quelconque des revendications précédentes, dans lequel ledit toner magnétique comprend en outre un isolant (4) mélangé avec celui-ci.

9. Toner magnétique selon l'une quelconque des revendications précédentes, dans lequel ledit toner magnétique comprend une matière magnétique en poudre (2) mélangée avec celui-ci, et dans lequel de la poudre métallique de l'un quelconque parmi le fer, le manganèse, le nickel, le cobalt, et le zinc est utilisée en tant que poudre magnétique, et dans lequel la taille moyenne de particule de la matière magnétique en poudre est au plus de 1 µm alors que la quantité ajoutée de celle-ci va de 20 à 60 % en poids.

10. Appareil destiné à mettre en oeuvre le traitement de surface du toner magnétique électrophotographique selon l'une quelconque des revendications précédentes, en supprimant uniformément l'agglomération du toner, l'appareil comprenant:
un moyen d'alimentation en toner (21) destiné à fournir le toner magnétique (22) avec une vitesse d'alimentation constante:
un moyen de pulvérisation (24) pour pulvériser et disperser le toner magnétique ;
un moyen d'alimentation en air comprimé (31) destiné à fournir de l'air comprimé (23) contenant le toner magnétique (22) audit moyen de pulvérisation (24) par un conduit de transport de toner (32) ;
un moyen de création d'air chaud (25) destiné à appliquer de l'air chaud (26) au toner magnétique (22) pulvérisé depuis ledit moyen de pulvérisation (24) ; et
un moyen de récupération de toner (28,29) destiné à récupérer le toner magnétique pulvérisé et dispersé dans l'air chaud (26), selon les revendications 1 à 9,
dans lequel le calibre de la partie formant ouverture du moyen de pulvérisation de toner (24) est plus petit que celui du conduit de transport de toner (32).

11. Appareil selon la revendication 10, dans lequel la pression de l'air comprimé est établie pour être de 5 000 à 30 000 kg/m² pour fournir le toner depuis ledit moyen d'alimentation en toner (21) jusqu' à l'entrée du moyen de pulvérisation (24), dans lequel la pression de l'air chaud est établie pour être de 15 000 à 50 000 kg/m², et dans lequel la température de l'air chaud est établie pour être dans la plage allant de 100 à 600°C.

12. Appareil selon la revendication 10 ou 11, comprenant en outre un tamis métallique (30) ayant une valeur d'ouverture allant de 30 à 200 µm au niveau de la partie ouverte du dit moyen de pulvérisation (24) pour supprimer l'agglomération du toner.

13. Appareil selon l'une quelconque des revendications 10 à 12, dans lequel le dit moyen de pulvérisation de toner comprend au moins une paire de buses de dispersion (24) avec de l'air comprimé, depuis lesquelles buses (24), le toner magnétique est pulvérisé avec l'air comprimé (23) dans la direction approximativement à 45 degrés.

14. Appareil selon le revendication 13, dans lequel les buses de dispersion (24) sont prévues pour être deux à des positions symétriques à droite et à gauche par rapport audit moyen de création d'air chaud (25).

15. Procédé de production de toner magnétique électrophotographique selon l'une quelconque des revendications 1 à 9, le procédé comprenant les étapes de :
malaxage d'une résine de liaison (1), des particules fines (2) d'une matière magnétique et des additifs (3,4,5),
pulvérisation des matières malaxées qui en résultent, tamisage de la matière pulvérisée, et
réalisation du traitement de surface de la matière tamisée dans son état dispersée par de l'air chaud pour accomplir la formation en sphères du toner magnétique,
caractérisé en ce que
le traitement de surface est effectué par fusion de la surface de la résine de liaison (1) de telle façon que chaque particule fine (2) de la matière magnétique qui est mise à nu sur la surface du toner magnétique est revêtue de la résine de liaison (1) et que les particules de toner sont formées en sphères simultanément et instantanément, à la condition que la pression de l'air comprimé soit établie pour être dans la plage de 5 000 à 30 000 kg/m², que la pression de l'air chaud soit dans la plage allant de 15 000 à 50 000 kg/m², et que la température de l'air chaud soit dans la plage allant de 100 à 600°C.

16. Dispositif électrophotograhique utilisant le toner magnétique électrophotographique selon l'une quelconque des revendications 1 à 9, le dispositif comprenant :
un moyen de développement qui comprend un élément rotatif de retenue de l'image latente électrostatique (101), lequel contient un aimant fixe (102) : un moyen formant citerne de toner (106) qui est en face d'une surface de l'élément de retenue d'image latente électrostatique (101) pour fournir le toner magnétique en faisant en sorte que l'aimant fixe (102) aspire magnétiquement le toner magnétique ; et un rouleau d'électrode (108) qui est situé à un intervalle spécifié par rapport à la surface de l'élément de retenue d'image latente électrostatique (101) et qui contient à l'intérieur un aimant (109) ;
un moyen de transfert (112) destiné à transférer le toner magnétique sur une matière de transfert (118) pour la visualisation de l'image latente électrostatique formée sur l'élément de retenue d'image latente électrostatique (101); un moyen de nettoyage (114,116) destiné à enlever de celui-ci le toner magnétique restant en partie après le transfert sur l'élément de retenue d'image latente électrostatique (101); et
un moyen de recyclage de toner (115) destiné à renvoyer à nouveau le toner magnétique qui a été enlevé par le moyen de nettoyage (114, 116) vers le procédé de développement, dans un but de recyclage ;
dans lequel le toner adhérant aux parties chargées du dit élément de retenue d'image latente électrostatique (101) est récupéré par le rouleau d'électrode (118), d'où il résulte qu'il reste sur le dit élément de retenue d'image latente électrostatique (101) une image de toner inversée négative-positive seulement en ce qui concerne les zones d'image.

17. Procédé électrophotographique utilisant le toner magnétique électrophographique selon l'une quelconque des revendications 1 à 9, le procédé comprenant les étapes de retenue d'une image latente électrostatique sur un élément de retenue d'image latente (101) ;
développement de l'image latente électrostatique retenue pour qu'elle soit visualisée au moyen du toner magnétique fourni en faisant en sorte que l'aimant fixe (102) aspire magnétiquement le toner ;
transfert de l'image développée avec le toner magnétique sur un élément de transfert (112) ;
nettoyage de l'élément de retenue d'image latente (101) pour enlever le toner magnétique qui reste partiellement après le procédé de transfert ; et
recyclage du toner pour renvoyer à nouveau le toner magnétique qui a été enlevé durant le procédé de nettoyage vers le procédé de développement, dans un but de recyclage.
